

## UNITED STATES PATENT OFFICE

ERNST BURI, OF ZURICH, SWITZERLAND

## PRINTING STUFF AND PRINTING METHOD

No Drawing. Application filed May 25, 1927, Serial No. 194,241, and in Germany May 25, 1926.

My invention relates to a dusting powder adapted to be reprinted; that is to say, a dusting powder having the quality of producing a printing surface by being transferred 5 to a lithographic stone, metal plate or the like. According to my invention the dusting powder contains lycopodium impregnated with soap.

The preparation of this dusting powder 10 may be performed in the following manner: 5 parts soap powder are added to 100 parts lycopodium moistened in water. The mixture obtained in this manner is well dried on a stove.

15 The preparation of a printing surface with the dried dusting powder obtained in this manner may be performed as follows: A paper having a surface of a swelling layer, for example gelatine, gum, glue or casein, is subjected 20 for a period of 1-2 minutes to luke-warm water. As a suitable paper for instance Autotype Co. London, double transfer paper may be employed. The paper will then be dried with a blotting-paper or handkerchief 25 and then the above described dusting powder is equally distributed on the paper by means of cottonwool. The powder containing lycopodium impregnated with soap has the quality of being capable of equal distribution on the swelling layer. The dusted paper is sensitized in a solution of 2-4% kalium-bichromate (potassium) then after being dried it is exposed for a period of 5-10 minutes under a negative until the copy is visible 30 in sharp outline. The paper is then subjected to the action of warm water so as to cause it to swell and then sprayed under strong water pressure, so that those parts not acted on by the light are washed away and a clear image 35 will appear. The paper is dried and then laid between wet papers until the image is quite flat. It is then put on an unprepared lithographic stone, metal plate or any other suitable printing surface and passed through a lithographic or other suitable printing press. By this means a fatty impression or copy of the impregnated lycopodium is obtained for 40 instance on the stone, which will be treated in the usual manner; that is to say, the fatty impression will be treated with gum, caustic

and ink. In this manner a perfected print- 45 able matrix is obtained. Numerous impres- sions of this matrix may be reproduced on the printing machine, by offset or the like.

The above described printing method 50 makes it possible to reproduce perfectly all 55 half tones without the employment of a screen, the corn of the dusting powder or printing stuff containing lycopodium, which 60 itself encloses a good deal of fat or oil, form- 65 ing a printable bearer.

Instead of dusting the powder on the swell- 70 ing layer by hand as described above, the im- 65 pregnated powder may be incorporated in an emulsion containing gelatine or other suit- 75 able substances, and this weak emulsion poured upon a suitable paper surface by machine in such manner that the impregnated lycopodium swims at the top of the surface, the layer 80 being then dried. From this point, the paper 70 is treated in the same manner as described above; that is to say, it is sensitized, exposed and so on. The paper so manufactured may 85 be produced in any desired length.

75 What I claim is:

A dusting powder adapted to be reprinted 90 containing lycopodium impregnated with soap.

In testimony whereof I have signed my 95 name to this specification.

ERNST BURI.

85

90

95

100